

# UNITED STATES PATENT OFFICE.

FRIEDRICH JOHANN HEINRICH ROEWER, OF HAMBURG, GERMANY.

## NITROGLYCERIN EXPLOSIVE.

No. 853,830.

Specification of Letters Patent.

Patented May 14, 1907.

Application filed July 25, 1905. Serial No. 271,252.

To all whom it may concern:

Be it known that I, FRIEDRICH JOHANN HEINRICH ROEWER, doctor of philosophy, chemist, a subject of the Grand Duke of Mecklenburg-Strelitz, residing at Hamburg, Germany, bei dem Zippelhause 18, have invented new and useful Improvements in Nitroglycerin Explosives, of which the following is a specification.

Various compounds have been proposed before for preventing or reducing the congealing tendency of nitroglycerin and nitroglycerin explosives, without, however, having come into practical use owing to inefficiency of purpose and detrimental effect upon the explosive force of nitroglycerin.

The present invention relates to monochlordinitroglycerin which I have discovered to be a compound suitable for reducing the congealing tendency of nitroglycerin, without lessening the force of the explosive. By adding 5 to 20 % monochlordinitroglycerin to nitroglycerin, explosives are obtained which in proportion to the amount of monochlordinitroglycerin added will either not congeal at all or at very low temperatures and without affecting the explosive force.

The mixture may be obtained either by adding the monochlordinitroglycerin to nitroglycerin or by nitrating monochlorhydrin and glycerin.

Monochlordinitroglycerin may be used without any disadvantage in the manufacture of non-gelatinized explosives; as for the manufacture of gelatinized explosives the addition of monochlordinitroglycerin facilitates the gelatinizing process and consequently a better gelatinous explosive results than with pure nitroglycerin.

Having now particularly described and ascertained the nature of my said invention and in what manner the same is to be performed, I declare that what I claim is:

A nitroglycerin explosive containing dinitro-monochlorhydrin, to protect the explosive from the danger of freezing, substantially as described.

In testimony whereof I have signed my name to this specification in the presence of two subscribing witnesses.

FRIEDRICH JOHANN HEINRICH ROEWER.

Witnesses:

ERNEST H. L. MUMMENHOFF,  
OTTO W. HELLMRICH.